

## UNITED STATES PATENT OFFICE

2,507,390

## BAKED CORES FOR USE IN METAL CASTING

Burgess P. Wallace, Brooklyn, N. Y., assignor to  
Whitehead Brothers Company, New York, N. Y.,  
a corporation of New JerseyNo Drawing. Application May 7, 1947,  
Serial No. 746,623

2 Claims. (Cl. 22—188)

1

This invention relates to the casting of metals and more especially to the production of destructible cores for use in casting difficultly oxidizable metals, such as grey iron, steel, bronze and their alloys.

The principal objects of the invention are the continuous and economical production of cores for such metal casting purposes as are capable of forming dimension-true holes in the resultant castings, the surfaces of which are perfectly smooth and entirely devoid of burnt-on sand grains, pits, cracks or other defects. Other objects of the invention are herein-after set forth.

In the manufacture of foundry cores, it is now customary to form the same by bonding together, into a core of the desired shape and size, particles of fusible, refractory substances, such as sand grains, for example, with organic binders as linseed oil, tung oil or the like, so-called cereal binders, synthetic resins, silicates, pitches and the like. The molded cores are then baked at an optimum temperature in an oven and usually, while still hot, though sometimes when cooled, a blacking coat of relatively insignificant thickness is either brushed or sprayed thereon or else the cores are dipped into a suspension of the blacking and allowed to drain. Not only are some of the sand or other fusible particles so bonded together in such cores either actually present in or in such close proximity to the surface of the core that during a casting operation the molten metal will reach the same and burn them into the surfaces of the resultant castings but the applied blacking coat, itself, also tends to render the cores untrue to the size and to pattern shape.

Further, the very fact that the blacking coat must of necessity be very fine to remain in suspension in the vehicle results in the undue clogging of the cores by the blacking with the consequent decrease in the permeability thereof to gases and volatilizable substances. Another disadvantage resulting from the use of blacking, is its tendency to peel or flake off on casting due to the different coefficients of expansion of the blacking and the uncoated core. Such tendency is materially aggravated if it be attempted to apply a blacking coat of more than

2

of carbon granules adhesively united with such a binder or which core, at least throughout the entire outer layer thereof to a depth at least about one-eighth inch below the surfaces thereof comprises such an agglomeration.

In carrying out my invention, I preferably proceed as follows:

Carbonaceous material having a fixed carbon value of about 45% at 700° C. and a residue when heated to 750° C. of about 10% by weight, such as a coke, for example, and selectively sized, in the customary manner, to the appropriate grain fineness, 10 between about 50 and 250 grain fineness number as defined by the Foundry Sand Grading Classification of the American Foundrymen's Association. By a judicious blending of the various sizes 15 of such grains in order to obtain the desired grain fineness number in the ground and sized coke, cores of any desired degree of permeability, such as aforesaid, can be obtained. Such carbonaceous materials as anthracite coal of low ash content, 20 coke, graphite and the like are especially desirable for the production of any improved cores. The blended grains of the carbonaceous base are then intimately admixed with a binder, such as one or more of the aforesaid standard binders, the 25 amount thereof being predetermined in the manner now customary to produce cores of the desired strength. The core is then molded and baked 30 in a standard core oven at an optimum temperature in the well-known manner such for example as described in Patents Nos. 973,574, 1,561,956 and 1,531,871, in order to dry out the water and moist 35 or soften the binder so that the carbon granules are thoroughly bound together so that the cores will possess the requisite hot strength when the 40 metal is poured about the same.

To cite a typical example of the procedure I have employed in producing my improved cores, a mixture is first prepared comprising a quantity of "72 hour" metallurgical coke, 45 prepared by heating coking coal for 72 hours in a by-product coke oven to about 1,000° F., the volatile at the coking temperature being

In making composite cores, it is preferable to mold or press the mulled mixture of carbon granules and binder into the form of a hollow matrix of the external shape desired with a wall thickness of at least about  $\frac{1}{8}$ " and desirably about  $\frac{1}{4}$ ", depending on the size of core desired and then the cavity in such matrix is filled with molding sand, gravel, cinders or other cheap filler very loosely bonded together with a binder such as aforesaid, whereupon the resulting shape is baked in the manner aforesaid. The baked composite core will have sufficient hot strength imparted thereto by the carbon matrix or shell thereof to be capable of resisting the erosive action of the hot metal while at the same time it will peel equally as well as if the entire core were composed of such agglomerated carbon granules.

It cannot be too strongly emphasized that my improved "solid" or "composite" cores have the combustible medium, i. e., the binder element, simultaneously baked integral with the other components of the core, as contra-distinguished from the ordinary core wherein the carbon blacking is usually applied as a wash of relatively insignificant thickness to a previously baked core composed of silica sand or like refractory grains bonded together and which wash is usually not baked so as to become an integral fused part of such cores.

My improved cores of either of the specified types thereof can be readily disintegrated and removed from the castings produced therewith. Since no blacking coat is required, there is a considerable saving in time and expense in the core making operation. These cores are of accurate dimensions, and due to the absence of any blacking coat there is nothing to peel off or flake off therefrom. Furthermore, in the "composite" type thereof the enveloping carbon layer or shell can be applied to any desired degree of thickness without deleteriously diminishing the gas permeability thereof. Since the core is composed either of carbon throughout agglomerated by the binder or at least to a very substantial depth below the surface, no molten metal can reach any sand or other frittable silicious particles during the casting operation such as invariably occurs when employing the ordinary sand cores above described. As a consequence, my improved cores perfectly face the area of the casting contacting therewith, thereby insuring the formation of dimension-true, clean holes whose walls are completely devoid of burnt-on sand or other fritted particles. Moreover, due to the fact that the blend of the grain sizes of the carbon employed can be of a definite predetermined or selected grain fineness number, it is possible to insure that such grains can be compacted to a maximum degree consistent with the gas permeability desired. The selected grains will have a maximum number of points of contact thus requiring but a minimum amount of binder to effectively cement the same together as compared with the amount ordinarily required in standard cores to produce a core of the desired strength or, in other words, my cores will possess an increased comparative strength as contrasted with the ordinary core if like amounts of binder are employed in both. My improved cores are suitable for use either in green, dry or baked molds.

The "composite core" above described is especially economical to produce, since the sand or like cheap filler comprising the center thereof constitutes its major portion as the surface layer

or shell is comparatively thin, being desirably one-quarter of an inch thick and not less than about one-eighth of an inch. Preferably the centers of these cores have a much weaker bond than the shell and accordingly they can be readily collapsed and disintegrated when it is desired to remove such cores from the casting and when the centers have been so disintegrated the shell can be easily collapsed and removed in fragments.

The organic binder in my improved cores, while it suffices to produce the requisite hot strength during casting of the metal, becomes consumed or decomposed to such an extent during such operation as to render the core easily disintegrable and consequently readily removable from the casting all in the manner now customary and in this respect functions quite differently from sodium silicate and like inorganic binders such as commonly employed in the manufacture of so-called permanent molds.

While I preferably employ but between about 2% and 3% of the organic binder, larger amounts, depending upon the nature of the particular binder employed, may be used but in no event should the amount thereof be sufficient to interfere with the requisite gas-permeability of the core or the ready disintegration and removal thereof from the casting.

30 The term matrix as used in the claims is intended to refer to the enveloping outer layer or shell of the composite core which envelops the filling thereof.

Various modifications of the herein described core composition and method, within the scope of the appended claims, may be made without departing from the spirit of my invention.

Having thus described my invention, I claim:

1. A baked core for use in casting metals, the same consisting essentially of a blend of grains of refractory carbon bonded together with a binder and which blend of carbon grains has a grain fineness number between about 50 and 250 as defined by the Foundry Sand Grading Classification of the American Foundrymen's Association.

2. A baked core for use in casting metals, the same consisting essentially, at least as to the outer layer thereof to a depth of about one-eighth of an inch beneath its outer surface, of a blend of grains of refractory carbon bonded together with a binder and which blend of carbon grains has a grain fineness number between about 50 and 250 as defined by the Foundry Sand Grading Classification of the American Foundrymen's Association.

BURGESS P. WALLACE.

#### REFERENCES CITED

60 The following references are of record in the file of this patent:

#### UNITED STATES PATENTS

| Number       | Name      | Date          |
|--------------|-----------|---------------|
| 65 174,356   | Darling   | Mar. 7, 1876  |
|              | 422,055   | Lytle         |
|              | 805,144   | Kuller        |
|              | 1,165,651 | Davis         |
|              | 1,316,471 | Acton et al.  |
| 70 1,467,112 | Lucier    | Sept. 4, 1923 |
|              | 1,775,576 | Waters        |
|              | 1,955,936 | Wallace       |
|              | 2,306,883 | Holmes        |
|              | 2,322,638 | Kleeman       |